

R. L. GILLIAM.  
PROCESS OF TREATING WOOD.  
APPLICATION FILED AUG. 26, 1914.

1,283,495.

Patented Nov. 5, 1918.



Witnesses

Benjamin Finkel  
P. N. Grant

Inventor  
Robert L. Gilliam  
By Lincoln Lincoln  
his Attorney

# UNITED STATES PATENT OFFICE.

ROBERT L. GILLIAM, OF COLUMBUS, OHIO, ASSIGNOR TO THE GILLIAM PROCESS COMPANY, OF COLUMBUS, OHIO, A CORPORATION OF OHIO.

## PROCESS OF TREATING WOOD.

1,283,495.

Specification of Letters Patent.

Patented Nov. 5, 1918.

Application filed August 26, 1914. Serial No. 858,743.

To all whom it may concern:

Be it known that I, ROBERT L. GILLIAM, a citizen of the United States, residing at Columbus, in the county of Franklin and State 5 of Ohio, have invented a certain new and useful Improvement in Processes of Treating Wood, of which the following is a specification.

The sap of some woods, and particularly 10 the sap of the wood of the sweet gum tree, consists in part of liquid and in part of a gummy or gelatinous substance. The liquid part is easily removed by subjecting the wood to a steaming or seasoning process but 15 the gelatinous part does not appear to be readily soluble or removable by the steam. It is the common experience with the lumber of the sweet gum tree, if not with the lumber of other species of tree, that it has upon 20 drying, after seasoning, a tendency to warp and twist. It has occurred to me that this warping and twisting is due to the retention of said gummy or gelatinous substance in the wood notwithstanding the steaming 25 process. After considerable experiment I discovered that if the steaming process be conducted in the presence of an alkali this gummy or gelatinous substance may be dissolved and the wood relieved of its tendency 30 to warp and twist and without apparent deleterious effect upon the fiber of the wood.

In carrying out my process I employ a treating chamber constructed substantially as hereinafter described and on the principle 35 illustrated in the accompanying drawings.

In said drawings—

Figure 1 is a vertical section.

Fig. 2 is a horizontal section of the chamber on the line  $x-x$  looking down.

Fig. 3 is a vertical section on the line  $y-y$  Fig. 2, on a larger scale to show a detail.

In the views 5 designates a room or chamber which is constructed so as to be reasonably steam tight and to have a suitable opening at 5<sup>a</sup> through which the lumber is passed into and out of the chamber. 6 is a basin, said basin being conveniently formed of concrete. In the floor of the basin is constructed a well 6<sup>a</sup>. 7 are pipes horizontally arranged within the room and connected with a header 8 located at the outer side of the structure. The pipes 7 are perforated as shown at 7<sup>a</sup> along their upper sides to afford exits for the steam into the chamber and 55 said pipes are perforated to permit the exit

of fluids. Connected with the bottom of the well 6<sup>a</sup> is a pipe 9 leading to a pump 10 which pumps the liquid from the well back into the pipes 7 from which it issues through the perforations into the chamber. The 60 liquid can be forced through a jetting device 11 arranged in the steam line 12. Any suitable means can be employed for agitating or circulating or distributing the steam and alkali to the wood as the particular means 65 shown do not constitute the present invention.

The lumber to be treated can be carried into the chamber by means of a car, the lumber being first "sticked" or piled on the car 70 so as to leave free spaces between it through which steam can circulate about the lumber.

In practice the green lumber or lumber to be treated is run into the chamber, but before closing the chamber and turning on 75 the steam I place in the basin 6 a quantity of an alkali, said alkali being preferably the ordinary commercial carbonate of soda because of its cheapness. Where the chamber has a working capacity of say thirty 80 thousand feet of lumber the first charge of soda according to my practice is about two hundred pounds and after this I supply the basin with about fifty pounds daily. After the soda has been supplied to the chamber 85

the door is closed tightly and the steam admitted through the pipes 7 to the chamber to maintain the temperature therein at about two hundred and twelve degrees Fahrenheit or at a temperature and for a period suffi- 90

cient to effect the seasoning of the lumber and the dissolution of the gummy or gelatinous substance before referred to. The duration of this treatment may vary according to the nature of the wood treated but the time necessary to effect the dissolution of the gummy or gelatinous substance in any particular wood may be readily ascertained by examining specimens of the wood from time to time. The sap or water of condensation 95 or both serve to dissolve the soda deposited in the basin. With some porous woods the dissolution of the gummy or gelatinous substance might be effected in as little as four or five hours or in the time employed in ordinary seasoning by the use of steam. The strength of the alkali might also make some difference in the time required. I have used my process in connection with the process for coloring the sap wood of the sweet gum 100

105

110

tree set forth in my Letters Patent of the United States, No. 1,084,266, dated January 13, 1914. In the process of that patent the wood of the sweet gum tree is colored or 5 tinted by subjecting it to the action of steam in the presence of iron. The process of treating the wood with alkali for the purpose herein described may be concurrent or simultaneous and in the same chamber with 10 the said treatment for coloring. In such concurrent or simultaneous treatment I have subjected the wood to treatment for forty-eight hours and have obtained a product having both the desired tint and freedom 15 from the aforesaid tendency to warp and twist. Where the treatment of the wood is directed to both coloring the wood and securing immunity against warping and twist-

ing and iron filings are used, such filings are put into the basin as set forth in my afore- 20 said former patent. It appears to be unim- portant that the time consumed for effecting a coloring may be greater than that neces- sary for effecting immunity to warping and 25 twisting.

What I claim is:

The process of treating the wood of the sweet gum tree for the purpose of prevent- 30 ing it from warping and twisting consisting in subjecting that wood to the action of steam mixed with a solution of an alkali in a confining chamber.

ROBERT L. GILLIAM.

Witnesses:

BENJAMIN FINCKEL,  
B. H. GRANT.